

Oct. 12, 1926.

1,602,835

J. D. REIFSNYDER

METHOD OF IMPREGNATING PAPER RECEPTACLES

Original Filed Dec. 31, 1921 2 Sheets-Sheet 1

Fig. 1.



Fig. 2.



Fig. 3.



James D. Reifsnnyder, INVENTOR  
Ward, Cossly and Smith,  
his ATTORNEYS.

Oct. 12, 1926.

1,602,835

J. D. REIFSNYDER

METHOD OF IMPREGNATING PAPER RECEPTACLES

Original Filed Dec. 31, 1921 2 Sheets-Sheet 2

*Fig. 4.*



*Fig. 5.*



*Fig. 6.*



INVENTOR.  
James D. Reifsnnyder  
BY Ward, Crosby and Smith,  
HIS ATTORNEYS.

## UNITED STATES PATENT OFFICE.

JAMES D. REILFSNYDER, OF BROOKLYN, NEW YORK, ASSIGNOR, BY MESNE ASSIGNMENTS, TO TULIP CUP CORPORATION, OF NEW YORK, N. Y., A CORPORATION OF DELAWARE.

## METHOD OF IMPREGNATING PAPER RECEPTACLES.

Original application filed December 31, 1921, Serial No. 526,259. Divided and this application filed January 14, 1924. Serial No. 686,223.

The invention relates to an improved method of impregnating paper receptacles. It is especially useful for the impregnation of individual paper drinking cups but may 5 also be used for the impregnation of other paper receptacles. This application is a division of my application improvements in impregnated individual paper drinking cup, Serial No. 526,259, filed December 31, 1921. 10 One of the objects of the invention is the provision of a simple and effective method of impregnating or treating individual paper cups, or other paper receptacles. Another object of the invention is the provision 15 of a method for impregnating a cup or other receptacle with a water proofing material which is not injurious and will not give an appreciable odor or taste when put to the lips, and which will not have an appreciable 20 coating of the indurating material, particularly on its outer surface. Another object is the provision of a method for so treating a cup or other receptacle as to render it especially useful for holding hot liquids. 25 The invention consists in the method of impregnating or treating paper receptacles hereinafter described according to the preferred manner of practicing the same and the invention will be more particularly 30 pointed out in the appended claims.

It has heretofore been the practice to make individual paper drinking cups both with plain and pleated walls, and to coat such cups by dipping them in melted paraffin, but cups thus made have a distinct coating of paraffin on the inner and outer surfaces, including the rim. This paraffin coating is unpleasant both to the touch of the lips and fingers, and is made more so 35 when any warm drink is poured into the cup. It may also produce spots on gloves. Furthermore, individual paper cups heretofore made are not suitable for holding hot liquids, since such cups will not hold their 40 forms and remain tight with fluids of a temperature of over about 120° Fah. Notwithstanding the decided coating of paraffin, these known cups are not useful for hot 45 drinks which should be dispensed or poured at a temperature of not much below 150° Fah. or higher so that the fluid will remain sufficiently hot while being drunk.

My improved cup when properly made

will withstand liquid at a temperature of about 170° Fah., and it is capable of doing 55 this while being free of any appreciable coating of the impregnating material.

Further objects and advantages of the invention will more fully appear from the following description taken in connection 60 with the accompanying drawings illustrating the preferred form of cup.

Referring to the drawings, Fig. 1 is a perspective view of a pleated cup impregnated by the method embodying my invention; 65

Fig. 2 is a sectional view of the same taken on line 2—2;

Fig. 3 is an enlarged section at the rim taken on line 3—3 of Fig. 2.

Figs. 4, 5 and 6 are diagrammatic views 70 indicating steps of the process.

The cup 1 shown in the drawings is a pleated cup shown and fully described in the United States Letters Patent No. 1,310,698, and is made of a suitable single 75 blank of material so as to provide pleated side walls 2 and a rolled rim 3. Cups of this character have three thicknesses of paper at certain portions thereof as shown in Fig. 3, where the pleats or folds occur. 80

While the invention is equally applicable to plain smooth surfaced cups, it is especially advantageous in impregnating pleated cups, because due to the folds and irregular surfaces, when such cups are dipped in paraffin in the usual way, i. e., in paraffin having a melting point of about 125° F., and at a temperature of about 175° F., they become coated with a very excessive amount 85 of paraffin.

In impregnating the cup according to my preferred process, I use a waxy impregnating material having a relatively high melting point and consisting preferably of a mixture of a vegetable wax with a high 90 melting point, such as carnauba having a melting point of about 180° Fah. and a high grade paraffin, i. e., one having a melting point of about 140° Fah. I preferably use about 20% by weight of the wax and 80% 95 of paraffin. This waxy mixture has a relatively high melting point of about 160° to 170° Fah.

I heat this mixture up to the relatively high temperature of about 250° Fah., then 100 apply it in liquid form to the cup, prefer-

ably only to a portion of the cup, so as not to get an excessive amount of the mixture on the cup, and then while the coating of the mixture on portions of the cup is yet hot, 5 I subject the cup to heat so as to cause the impregnating liquid to spread over the whole surface of the cup and impregnate the same. I preferably apply the impregnating liquid to the inside of the cup by pouring it into the 10 cup, sufficient to fill the cup from one-eighth to one-quarter full, then immediately empty the liquid from the cup while giving the cup a twist of from one-half to a full revolution. This causes the liquid to flow over the inner 15 surface in a spiral-like path from the bottom toward the rim, so as to leave the liquid distributed over only portions of the cup extending from the bottom to the rim. The cup is then passed into an oven kept at a 20 temperature of about 180° to 200° Fah., as a lower limit, to which temperature the cup is subjected for about 45 seconds to a minute. The temperature of the oven should, of course, be kept below that at which discol- 25 oring or charring of the cup takes place, this temperature varying with the length of the oven and the time required for the cups to pass through the same. This keeps the liquid thin so that it will readily spread over the 30 entire surface and thoroughly impregnate the shell of the cup.

In this manner I can produce a cup having substantially no coating on the outside, and little or none on the inside, and yet having the shell of the cup so thoroughly impregnated with the waterproofing material of relatively high melting point that it will withstand hot liquids at a temperature of about 170° Fah.

40 I have found that once an excess of impregnating fluid is applied to the paper shell of the cup, it is very difficult to drain it off, and if left on it produces the undesirable coating on the surface of the cup. This is 45 probably the reason for the coating found on cups simply dipped in hot paraffin. But by applying the liquid on only portions of the cup and keeping the liquid hot, the uncoated part of the paper cup shell will 50 absorb and take up substantially all of the liquid on the coated portions of the cup so that the liquid will spread all over and thoroughly impregnate the shell to such an extent as to leave substantially no excess of the impregnating solution on the surface of the cup. I have found that when this process is 55 properly carried out and where a proper waxy material with a relatively high melting point such as that described, is used, the cup is so thoroughly impregnated that it 60 will hold liquids at a temperature of about 170° Fah. and yet the surface of the cup is substantially free of any surface coating so that the cup is dry and clean to 65 the touch rather than having an oily waxy

feel; and the outer surface, even when scraped with a sharp edge, shows no coating. The cup is of a pleasing white uniform color, slightly translucent, and is, by the impregnation, rendered stiffer and firmer than 70 it would otherwise be, and this without having the pleats gummed together by the impregnating material, as has been the practice.

The steps of the process are indicated diagrammatically in Figs. 4, 5 and 6 of the drawings in which Fig. 4 shows a measured relatively small quantity of hot impregnating liquid being poured from a spout 4 into the cup 1. In Fig. 5 the cup 1 is shown as somewhat tilted during the inversion of the same to pour out the surplus liquid, the cup also being given a twisting motion or motion of rotation about its own vertical axis during the tilting, the liquid in the cup moving in separated spiral paths over the inner surface of the cup during this motion as is indicated by the dotted lines 5. In Figure 6 the cup is shown as placed within an oven 6 whereby heat is supplied to keep the impregnating material on the inner surface of the cup liquid, to allow the same to spread to cover the entire inner surface and to be absorbed within the body of the cup.

While I have described the preferred method of impregnating a cup or other paper receptacle, it will be understood by those skilled in the art, after understanding my invention, that modifications may be made therein without departing from the spirit or scope of the invention, and I aim in the appended claims to cover all such modifications as come within the spirit or scope of the invention.

It is noted that suitable apparatus by which the method herein described and claimed may effectively be practiced is described and claimed in my co-pending application Serial No. 532,181, filed January 27, 1922, entitled "Apparatus for treating paper cups and the like."

What I claim is:

1. The method of impregnating thin individual paper cups which comprises, applying a hot impregnating liquid to separated portions only of the cup surface, and subjecting the cup to an atmosphere sufficiently hot to keep the impregnating material on the cup in a liquid condition and permitting the same to spread over the surface and impregnate the cup.

2. The method of impregnating individual paper cups which comprises, applying a hot impregnating liquid of relatively high melting point, at a temperature of not less than about 200° F., to separated portions only of the cup surface, and subjecting the cup to an atmosphere sufficiently hot to keep the impregnating material on the cup in a liquid

condition and permitting the same to spread over the surface and impregnate the cup.

3. Method of impregnating thin paper receptacles which comprises pouring a hot impregnating liquid into the receptacle to only partly fill it, and then emptying the material from the receptacle while giving the receptacle a twisting motion so as to coat a spiral-like portion of the receptacle, and then passing the receptacle into an oven to maintain the impregnating fluid hot to effect spreading of the liquid over the shell of the receptacle and impregnation of the shell.

4. The method of impregnating thin paper receptacles which comprises, applying a hot impregnating liquid to the inside only

of the receptacle, quickly inverting the receptacle to pour out the surplus, and then subjecting the receptacle to heat while the impregnating material on the inner surface 20 thereof is still hot.

5. The method of impregnating thin paper cups which comprises, pouring a measured relatively small quantity of hot impregnating liquid into the cup, tilting the cup to 25 empty it and at the same time giving it a different motion so that the liquid therein will flow laterally relatively to the cup.

In testimony whereof I have signed my name to this specification.

JAMES D. REIFSNYDER.